# EUROPEAN PATENT SPECIFICATION

(11) **EP 1 817 166 B1**
(45) Date of publication and mention of the grant of the patent: **20.01.2010**
(21) Application number: 05789446.1
(22) Date of filing: 15.09.2005
(51) Int. Cl.: B41C 1/10, B41M 5/36

(54) **METHOD OF MAKING LITHOGRAPHIC PRINTING PLATES**
VERFAHREN ZUR HERSTELLUNG VON LITHOGRAPHIE-DRUCKPLATTEN
PROCEDE DE PRODUCTION DE PLAQUES D'IMPRESSION LITHOGRAPHIQUE

(30) Priority: 01.10.2004 EP 04104827; 12.10.2004 US 617694 P
(43) Date of publication of application: 15.08.2007
(73) Proprietor: AGFA GRAPHICS NV, 2640 Mortsel (BE)
(72) Inventor: VERMEERSCH, Joan, AGFA-GEVAERT, B-2640 Mortsel (BE); VAN AERT, Huub, AGFA-GEVAERT, B-2640 Mortsel (BE)
(74) Representative: Goedeweeck, Rudi
(86) International application number: PCT/EP2005/054585
(87) International publication number: WO 2006/037716

(56) References cited:
- EP-A- 0 849 091
- EP-A- 1 048 458
- EP-A- 1 208 972
- EP-A- 1 342 568
- EP-A- 1 366 898
- EP-A1- 1 614 539
- EP-A1- 1 614 540
- EP-A2- 1 614 538
- WO-A-99/37481
- WO-A-02/051636
- US-A1- 2003 235 776

## Description

### FIELD OF THE INVENTION

The present invention relates to a method for making a lithographic printing plate whereby a printing plate precursor, having an improved sensitivity, is image-wise exposed and developed with a gum solution.

### BACKGROUND OF THE INVENTION

In lithographic printing, a so-called printing master such as a printing plate is mounted on a cylinder of the printing press. The master carries a lithographic image on its surface and a printed copy is obtained by applying ink to said image and then transferring the ink from the master onto a receiver material, which is typically paper. In conventional, so-called "wet" lithographic printing, ink as well as an aqueous fountain solution (also called dampening liquid) are supplied to the lithographic image which consists of oleophilic (or hydrophobic, i.e. ink-accepting, water-repelling) areas as well as hydrophilic (or oleophobic, i.e. water-accepting, ink-repelling) areas. In so-called "driographic" printing, the lithographic image consists of ink-accepting and ink-abhesive (ink-repelling) areas and during driographic printing, only ink is supplied to the master.

Printing masters are generally obtained by the so-called computer-to-film (CtF) method wherein various pre-press steps such as typeface selection, scanning, color separation, screening, trapping, layout and imposition are accomplished digitally and each color selection is transferred to graphic arts film using an imagesetter. After processing, the film can be used as a mask for the exposure of an imaging material called plate precursor and after plate processing, a printing plate is obtained which can be used as a master. Since about 1995, the so-called 'computer-to-plate' (CtP) method has gained a lot of interest. This method, also called 'direct-to-plate', bypasses the creation of film because the digital document is transferred directly to a plate precursor by means of a so-called plate-setter.

Especially thermal plates, which are sensitive to heat or infrared light, are widely used in computer-to-plate methods because of their daylight stability. Such thermal materials may be exposed directly to heat, e.g. by means of a thermal head, but preferably comprise a compound that converts absorbed light into heat and are therefore suitable for exposure by lasers, especially infrared laser diodes. The heat, which is generated on image-wise exposure, triggers a (physico-)chemical process, such as ablation, polymerization, insolubilization by cross-linking of a polymer, decomposition, or particle coagulation of a thermoplastic polymer latex, and after optional processing, a lithographic image is obtained. Many thermal plate materials are based on heat-induced ablation. A problem associated with ablative plates is the generation of debris which is difficult to remove and may disturb the printing process or may contaminate the exposure optics of the plate-setter. As a result, such ablative plates require a processing step for removing the debris from the exposed material.

EP 1 075 941 discloses a radiation-sensitive printing plate precursor wherein a photo-heat conversion agent is incorporated and wherein the photo-heat conversion agent is a particulate metal oxide comprising an organic photo-heat conversion compound encapsulated therein.

US 4,841,040 discloses a novel phosphated, oxidized starch having a molecular weight of about 1,500 to about 40, 000 u (or Daltons), a carboxyl degree of substitution of 0.30 to 0.96, and a phosphate degree of substitution of from about 0.002 to about 0.005, which is useful as a replacement for gum arabic in gumming and fountain solutions for lithography.

US 4,245,031 discloses photopolymerizable compositions containing a polymer having a plurality of salt-forming groups, two specific ethylenically unsaturated compounds and a radiation-sensitive, free-radical generating system. The compositions provide photopolymerizable elements which have outstanding photospeeds and are relatively insensitive to oxygen.

EP 770 497 discloses a method wherein an imaging material comprising an image-recording layer of a hydrophilic binder, a compound capable of converting light to heat and hydrophobic thermoplastic polymer particles, is image-wise exposed, thereby inducing coalescence of the polymer particles and converting the image-recording layer into an hydrophobic phase which defines the printing areas of the printing master. Subsequently the image-wise exposed precursor is developed by rinsing it with plain water or an aqueous liquid.

EP 1 366 898 discloses a printing method comprising the steps of (i) applying a coating including hydrophobic thermoplastic polymer particles onto a support having a surface roughness Ra of less than 0.45 mm, (ii) image-wise exposing and (iii) processing the obtained precursor. After the print run, the support is recycled - by removing the hydrophobic printing areas - and re-used in a next cycle of coating, exposing, processing and printing.

EP 514 145 discloses a radiation-sensitive plate which comprises a coating comprising core-shell particles having a water insoluble heat softenable core component and a shell component which is soluble or swellable in aqueous alkaline medium. The radiation causes selected particles to coalescence, at least partially, to form an image and the non-coalesced particles are then selectively removed by means of an aqueous alkaline developer.

In EP 1614538, EP 1614539 and EP 1614540, documents under A 54(3), a lithographic printing plate precursor is disclosed which comprises on a hydrophilic support a coating comprising an image-recording layer which comprises hydrophobic thermoplastic polymer particles having an average particle size ranging from 45 to 63 nm and wherein the amount of thermoplastic polymer particles is at least 70 % by weight relative to the image-recording layer. After exposure, the precursors are developed with an alkaline developing solution whereby the non-image areas of the coating are removed.

EP 1 342 568 discloses a method wherein an imaging material comprising an image-recording layer of a hydrophilic binder, a compound capable of converting light to heat and hydrophobic thermoplastic polymer particles, is image-wise exposed, thereby inducing coalescence of the polymer particles and converting the image-recording layer into an hydrophobic phase which defines the printing areas of the printing master. Subsequently the image-wise exposed precursor is processed with a gum solution, thereby developing and gumming the plate in a single step. In this single step process, the image-recording layer at the non-exposed areas is removed with the gum solution from the support, revealing the hydrophilic surface of the support, also called "clean-out", and simultaneously the hydrophilic surface in these non-image areas is protected from contamination (fingerprints, fats, oils, dust, oxidation, etc.) by the gum.

A plate system :AZURA (trademark from AGFA), that works according to the above mechanism, has been introduced to the market in May 2004. A problem associated with this printing plate precursor is the low sensitivity, i.e. the plate precursor needs a higher energy dose on image-wise exposure to obtain a sufficient coalescence of the polymer particles such that the non-exposed areas can be removed by the gum solution without affecting the exposed areas. This implies the plate requires a longer exposure time and/or a higher power laser, resulting in a lower speed. If a printing plate precursor is exposed with an energy dose which is too low in relation with its sensitivity, a lower quality for the lithographic printing properties can be obtained. This lower quality may result in a lower resolution, i.e. the precursor with the reduced sensitivity is not capable of rendering fine dots of a high resolution screen after exposure with the lower energy dose and after developing with a gum solution. Also the run length of the plate may be reduced as a result of a too low energy dose in relation with the sensitivity of the precursor due to an insufficient coalescence of the polymer particles in the exposed areas. It is further important for a high quality printing plate that the hydrophobic-hydrophilic differentiation in the coating is sufficient such that an excellent clean-out can be obtained, i.e. the non-exposed areas are completely removed from the support revealing the hydrophilic surface without affecting the exposed areas. An insufficient clean-out may further result in toning on the press, i.e. an undesirable increased tendency of ink-acceptance in the non-image areas.

### SUMMARY OF THE INVENTION

It is an object of the present invention to provide a method for making a lithographic printing plate wherein the lithographic printing plate precursor has an improved sensitivity and wherein the plates exhibit an excellent clean-out, no toning, and a high printing run length.

According to the present invention, this object is realized by the method of preparing a lithographic printing plate comprising the steps of
- providing a lithographic printing plate precursor comprising
   (i) a support having a hydrophilic surface or which is provided with a hydrophilic layer,
   (ii) on said support, a coating comprising an image recording layer, said layer comprising hydrophobic thermoplastic polymer particles and a hydrophilic binder, said coating further comprising a pigment, present in said image recording layer or in an additional layer of said coating,
- image-wise exposing said coating, thereby inducing coalescence of the thermoplastic polymer particles at the exposed areas of the image recording layer,
- developing the precursor by applying a gum solution to the coating, thereby removing the non-exposed areas of the image recording layer from the support, and
- optionally, baking the developed precursor,
wherein said hydrophobic thermoplastic polymer particles have an average particle size between 40 nm and 63 nm,
wherein the amount of the hydrophobic thermoplastic polymer particles in the image recording layer is more than 70 % and less than 85 % by weight, relative to the image recording layer, and
wherein said pigment has a hydrophilic surface and provides a visible image after image-wise exposing and developing with the gum solution.

Specific embodiments of the present invention are defined in the dependent claims. Further advantages and embodiments of the present invention will become apparent from the following description.

### DETAILED DESCRIPTION OF THE INVENTION

In the present description, all concentrations of compounds are expressed as percentage by weight, hereinafter also referred to as "wit.%" or "% wt", unless otherwise indicated.

The lithographic printing plate precursor used in the method of the present invention is negative-working and develops a lithographic image consisting of hydrophobic and hydrophilic areas at the exposed and non-exposed areas respectively. The hydrophobic areas and the hydrophilic areas are respectively defined by the coating and by the support, which has a hydrophilic surface or is provided with a hydrophilic layer.

The support may be a sheet-like material such as a plate or it may be a cylindrical element such as a sleeve which can be slid around a print cylinder of a printing press. Preferably, the support is a metal support such as aluminum or stainless steel.

A particularly preferred lithographic support is a grained and anodized aluminum support. Graining an anodizing of aluminum supports is well known. The grained aluminum support used in the material of the present invention is preferably an electrochemically grained support. The acid used for graining can be e.g. nitric acid or sulfuric acid. The acid used for graining preferably comprises hydrogen chloride. Also mixtures of e.g. hydrogen chloride and acetic acid can be used. The relation between electrochemical graining and anodizing parameters such as electrode voltage, nature and concentration of the acid electrolyte or power consumption on the one hand and the obtained lithographic quality in terms of Ra and anodic weight (g/m² of Al₂O₃ formed on the aluminum surface) on the other hand is well known. More details about the relation between various production parameters and Ra or anodic weight can be found in e.g. the article "Management of Change in the Aluminium Printing Industry" by F. R. Mayers, published in the ATB Metallurgie Journal, volume 42 nr. 1-2 (2002) pag. 69.

The anodized aluminum support may be subject to a so-called post-anodic treatment to improve the hydrophilic properties of its surface. For example, the aluminum support may be silicated by treating its surface with a sodium silicate solution at elevated temperature, e.g. 95°C. Alternatively, a phosphate treatment may be applied which involves treating the aluminum oxide surface with a phosphate solution that may further contain an inorganic fluoride. Further, the aluminum oxide surface may be rinsed with a citric acid or citrate solution. This treatment may be carried out at room temperature or may be carried out at a slightly elevated temperature of about 30 to 50°C. A further interesting treatment involves rinsing the aluminum oxide surface with a bicarbonate solution. Still further, the aluminum oxide surface may be treated with polyvinylphosphonic acid, polyvinylmethylphosphonic acid, phosphoric acid esters of polyvinyl alcohol, polyvinylsulfonic acid, polyvinylbenzenesulfonic acid, sulfuric acid esters of polyvinyl alcohol, and acetals of polyvinyl alcohols formed by reaction with a sulfonated aliphatic aldehyde.

Another useful post-anodic treatment may be carried out with a solution of polyacrylic acid or a polymer comprising at least 30 mol% of acrylic acid monomeric units, e.g. GLASCOL D15, a polyacrylic acid, commercially available from ALLIED COLLOIDS.

The support can also be a flexible support, which may be provided with a hydrophilic layer, hereinafter called 'base layer'. The flexible support is e.g. paper, plastic film or aluminum. Preferred examples of plastic film are polyethylene terephthalate film, polyethylene naphthalate film, cellulose acetate film, polystyrene film, polycarbonate film, etc. The plastic film support may be opaque or transparent.

The base layer is preferably a cross-linked hydrophilic layer obtained from a hydrophilic binder cross-linked with a hardening agent such as formaldehyde, glyoxal, polyisocyanate or a hydrolyzed tetra-alkylorthosilicate. The latter is particularly preferred. The thickness of the hydrophilic base layer may vary in the range of 0.2 to 25 µm and is preferably 1 to 10 µm. More details of preferred embodiments of the base layer can be found in e.g. EP-A 1 025 992.

The coating provided on the support comprises an image-recording layer which contains hydrophobic thermoplastic polymer particles.

In accordance with the present invention, the hydrophobic polymer particles have a number average particle size between 40 nm and 63 nm, preferably between 45 nm and 63 nm, more preferably between 45 nm and 59 nm. Herein, the particle size is defined as the particle diameter, measured by Photon Correlation Spectrometry, also known as Quasi-Elastic or Dynamic Light-Scattering. This technique is a convenient method for measuring the particle size and the values of the measured particle size match well with the particle size measured with transmission electronic microscopy (TEM) as disclosed by Stanley D. Duke et al. in Calibration of Spherical Particles by Light Scattering, in Technical Note-002B, May 15, 2000 (revised 1/3/2000 from a paper published in Particulate Science and Technology 7, p. 223-228 (1989). As mentioned in the Examples, the average particle size can be measured with a Brookhaven BI-90 analyzer, commercially available from Brookhaven Instrument Company, Holtsville, NY,USA.

In accordance to another embodiment of the present invention, the amount of hydrophobic thermoplastic polymer particles contained in the image-recording layer is more than 70 wt.% and less than 85 wt.%, preferably between 75 wt.% and 84 wt.%, more preferably between 77 wt.% and 83 wt.%.

The hydrophobic thermoplastic polymer particle comprises a hydrophobic polymer. Specific examples of suitable hydrophobic polymers are e.g. polyethylene, poly(vinyl chloride), poly(methyl (meth)acrylate), poly(ethyl (meth)acrylate), poly(vinylidene chloride), poly(meth)acrylonitrile, poly(vinyl carbazole), polystyrene or copolymers thereof. Polystyrene and poly(meth)acrylonitrile or their derivatives are highly preferred embodiments. According to such preferred embodiments, the polymer comprises at least 50 wt.% of polystyrene, and more preferably at least 60 wt.% of polystyrene. In order to obtain sufficient resistivity towards organic chemicals, such as the hydrocarbons used in plate cleaners, the polymer preferably comprises at least 5 wt.%, more preferably at least 30 wt.% of nitrogen containing monomeric units or of units which correspond to monomers that are characterized by a solubility parameter larger than 20, such as (meth)acrylonitrile. Suitable examples of such nitrogen containing monomeric units are disclosed in EP-A 1 219 416. According to the most preferred embodiment, the polymer is a copolymer consisting essentially of styrene and acrylonitrile units in a weight ratio between 1:1 and 5:1 (styrene:acrylonitrile), e.g. in a 2:1 ratio.

The weight average molecular weight of the thermoplastic polymer particles may range from 5,000 to 1,000,000 g/mol.

The hydrophobic thermoplastic polymer particles are present as a dispersion in an aqueous coating liquid of the image-recording layer and may be prepared by the methods disclosed in US 3,476,937. Another method especially suitable for preparing an aqueous dispersion of the thermoplastic polymer particles comprises:
- dissolving the hydrophobic thermoplastic polymer in an organic water immiscible solvent,
- dispersing the thus obtained solution in water or in an aqueous medium and
- removing the organic solvent by evaporation.
   The image-recording layer further comprises a hydrophilic binder. Specific examples of hydrophilic binders are homopolymers and copolymers of vinyl alcohol, acrylamide, methylol acrylamide, methylol methacrylamide, acrylic acid, methacrylic acid, hydroxyethyl acrylate, hydroxyethyl methacrylate or maleic anhydride/vinylmethylether copolymers. The hydrophilicity of the (co)polymer or (co)polymer mixture used is preferably the same as or higher than the hydrophilicity of polyvinyl acetate hydrolyzed to at least an extent of 60 percent by weight, preferably 80 percent by weight.
   In accordance with another embodiment of the present invention, the image-recording layer has preferably a coating weight between 0.45 and 0.83 g/m², more preferably between 0.50 and 0.80 g/m², most preferably 0.55 and 0.75 g/m².
   The coating may comprise, beside the image recording layer, one or more additional layer(s). Such an additional layer can be e.g. an adhesion-improving layer between the image-recording layer and the support; or a light-absorbing layer comprising one or more of the above compounds that are capable of converting infrared light into heat; or a covering layer which is removed during processing with a gum solution.
   The image-recording layer or an additional layer further contains a pigment having a hydrophilic surface and providing a visible image after image-wise exposing and developing with a gum solution. The hydrophilicity of the surface may be formed by the presence of hydrophilic groups, such as anionic or non-ionic groups, on the surface of the pigment particle. A hydrophilic surface may be formed by surface treatment, coating or adsortion of compounds such as hydrophilic polymers, reactive materials (e.g. silane coupling agent, an epoxy compound, polyisocyanate, or the like), surfactants (e.g. anionic or non-ionic surfactants) or water soluble salts (e.g. salts of phosphoric acid). Typical hydrophilic polymers are polymers or copolymers having anionic groups such as carboxylic acid, sulphonic acid, phosphonic acid, phosphoric acid, or salts thereof, or having a polyalkylene oxide group such as polyethyleneoxide. Specific examples of colorants are defined in the non-published EP-A 03 103 827. In accordance with the present invention, carbon dispersions in water such as CAB O JET 200, commercially available from CABOT, are preferred, and phthalocyanine pigment dispersions in water such as CAB O JET 250, commercially available from CABOT, are most preferred.
   The image-recording layer or an additional layer may also contain other ingredients such as additional binders, surfactants, development inhibitors or accelerators, and especially an IR-absorbing agent. An IR-absorbing agent is a compound capable of converting infrared light into heat. Particularly useful light-to-heat converting compounds or IR-absorbing agents are for example infrared dyes, carbon black, metal carbides, borides, nitrides, carbonitrides, bronze-structured oxides, and conductive polymer dispersions such as polypyrrole, polyaniline or polythiophene dispersions.
   In accordance with a preferred embodiment of the present invention, the coating comprises an IR-absorbing agent, more preferably the image recording layer comprises an IR-absorbing agent, and most preferably the image recording layer comprises an IR-absorbing agent in an amount of at least 6 % by weight relative to the image recording layer.
   The printing plate precursors used in the present invention are exposed to heat or to infrared light, e.g. by means of an infrared laser or LEDs. Preferably, a laser emitting near infrared light having a wavelength in the range from about 700 to about 1500 nm is used, e.g. a semiconductor laser diode, a Nd:YAG or a Nd:YLF laser. The required laser power depends on the sensitivity of the image-recording layer, the pixel dwell time of the laser beam, which is determined by the spot diameter (typical value of modern plate-setters at 1/e² of maximum intensity : 10-25 µm), the scan speed and the resolution of the exposure apparatus (i.e. the number of addressable pixels per unit of linear distance, often expressed in dots per inch or dpi; typical value : 1000-4000 dpi). Two types of laser-exposure apparatuses are commonly used : internal (ITD) and external drum (XTD) plate-setters. ITD plate-setters for thermal plates are typically characterized by a very high scan speed up to 500 m/sec and may require a laser power of several Watts. XTD plate-setters for thermal plates having a typical laser power from about 200 mW to about 1 W operate at a lower scan speed, e.g. from 0.1 to 10 m/sec.
   Due to the heat generated during the exposure step, the hydrophobic thermoplastic polymer particles fuse or coagulate so as to form a hydrophobic phase which corresponds to the printing areas of the printing plate. Coagulation may result from heat-induced coalescence, softening or melting of the thermoplastic polymer particles. There is no specific upper limit to the coagulation temperature of the thermoplastic hydrophobic polymer particles, however the temperature should be sufficiently below the decomposition temperature of the polymer particles. Preferably the coagulation temperature is at least 10°C below the temperature at which the decomposition of the polymer particles occurs. The coagulation temperature is preferably higher than 50°C, more preferably above 100°C.
   In the development step, the non-exposed areas of the image-recording layer are removed by supplying a gum or baking gum solution without essentially removing the exposed areas, i.e. without affecting the exposed areas to an extent that renders the ink-acceptance of the exposed areas inacceptable. The development by supplying a gum or baking gum may be combined with mechanical rubbing, e.g. by a rotating brush. The gum or baking gum solution can be applied to the plate e.g. by rubbing in with an impregnated pad, by dipping, (spin-)coating, spraying, pouring-on, either by hand or in an automatic processing apparatus. After applying the baking gum solution, the plate can be dried before baking or is dried during the baking process itself. The baking process can proceed at a temperature above the coagulation temperature of the thermoplastic polymer particles, e.g. between 100°C and 230°C for a period of 5 to 40 minutes. For example the exposed and developed plates can be baked at a temperature of 230°C for 5 minutes, at a temperature of 150°C for 10 minutes or at a temperature of 120°C for 30 minutes. Baking can be done in conventional hot air ovens or by irradiation with lamps emitting in the infrared or ultraviolet spectrum.
   A gum solution is typically an aqueous liquid which comprises one or more surface protective compounds that are capable of protecting the lithographic image of a printing plate against contamination, e.g. by oxidation, fingerprints, fats, oils or dust, or damaging, e.g. by scratches during handling of the plate. Suitable examples of such compounds are film-forming hydrophilic polymers or surfactants. The layer that remains on the plate after treatment with the gum solution preferably comprises between 0.1 and 20 g/m² of the surface protective compound.
   A gum solution is normally supplied as a concentrated solution which is diluted by the end user with water before use. In the present description, all concentrations of compounds present in the gum solution are expressed as percentage by weight (wt.% or % w/w) relative to the non-diluted gum solution, unless otherwise indicated.
   Preferred polymers for use as protective compound in the gum solution are gum arabic, pullulan, cellulose derivatives such as carboxymethylcellulose, carboxyethylcellulose or methylcellulose, (cyclo)dextrin, poly(vinyl alcohol), poly(vinyl pyrrolidone), polysaccharide, homo- and copolymers of acrylic acid, methacrylic acid or acrylamide, a copolymer of vinyl methyl ether and maleic anhydride, a copolymer of vinyl acetate and maleic anhydride or a copolymer of styrene and maleic anhydride. Highly preferred polymers are homo- or copolymers of monomers containing carboxylic, sulfonic or phosphonic groups or the salts thereof, e.g. (meth)acrylic acid, vinyl acetate, styrene sulfonic acid, vinyl sulfonic acid, vinyl phosphonic acid or acrylamidopropane sulfonic acid.
   Examples of surfactants for use as surface protective agent include anionic or nonionic surfactants. The gum solution may also comprise one or more of the above hydrophilic polymers as surface protective agent and, in addition, one or more surfactants to improve the surface properties of the coated layer. The surface tension of the gum solution is preferably from 40 to 50 mN/m.
   The gum solution comprises preferably an anionic surfactant, more preferably an anionic surfactant whereof the anionic group is a sulphonic acid group.
   Examples of the anionic surfactant include aliphates, abietates, hydroxyalkanesulfonates, alkanesulfonates,
   dialkylsulfosuccinates, straight-chain alkylbenzenesulfonates, branched alkylbenzenesulfonates, alkylnaphthalenesulfonates, alkylphenoxypolyoxyethylenepropylsulfonates, salts of polyoxyethylene alkylsulfophenyl ethers, sodium N-methyl-N-oleyltaurates, monoamide disodium N-alkylsulfosuccinates, petroleum sulfonates, sulfated castor oil, sulfated tallow oil, salts of sulfuric esters of aliphatic alkylesters, salts of alkylsulfuric esters, sulfuric esters of polyoxyethylenealkylethers, salts of sulfuric esters of aliphatic monoglycerides, salts of sulfuric esters of polyoxyethylenealkylphenylethers, salts of sulfuric esters of polyoxyethylenestyrylphenylethers, salts of alkylphosphoric esters, salts of phosphoric esters of polyox-yethylenealkylethers, salts of phosphoric esters of polyoxyethylenealkylphenylethers, partially saponified compounds of styrenemaleic anhydride copolymers, partially saponified compounds of olefin-maleic anhydride copolymers, and naphthalenesulfonateformalin condensates. Particularly preferred among these anionic surfactants are dialkylsulfosuccinates, salts of alkylsulfuric esters and alkylnaphthalenesulfonates.
   Specific examples of suitable anionic surfactants include sodium dodecylphenoxybenzene disulfonate, the sodium salt of alkylated naphthalenesulfonate, disodium methylene-dinaphtalene-disulfonate, sodium dodecyl-benzenesulfonate, sulfonated alkyl-diphenyloxide, ammonium or potassium perfluoroalkylsulfonate and sodium dioctyl-sulfosuccinate.
   Suitable examples of the nonionic surfactants include polyoxyethylene alkyl ethers, polyoxyethylene alkyl phenyl ethers, polyoxyethylene polystyryl phenyl ethers, polyoxyethylene polyoxypropylene alkyl ethers, polyoxyethylene polyoxypropylene block polymers, partial esters of glycerinaliphatic acids, partial esters of sorbitanaliphatic acid, partial esters of pentaerythritolaliphatic acid, propyleneglycolmonoaliphatic esters, partial esters of sucrosealiphatic acids, partial esters of polyoxyethylenesorbitanaliphatic acid, partial esters of polyoxyethylenesorbitolaliphatic acids, polyethyleneglycolaliphatic esters, partial esters of poly-glycerinaliphatic acids, polyoxyethylenated castor oils, partial esters of polyoxyethyleneglycerinaliphatic acids, aliphatic diethanolamides, N,N-bis-2-hydroxyalkylamines, polyoxyethylene alkylamines, triethanolaminealiphatic esters, and trialkylamine oxides. Particularly preferred among these nonionic surfactants are polyoxyethylene alkylphenyl ethers and poloxyethylene-polyoxypropylene block polymers. Further, fluorinic and siliconic anionic and nonionic surfactants may be similarly used.
   Two or more of the above surfactants may be used in combination. For example, a combination of two or more different anionic surfactants or a combination of an anionic surfactant and a nonionic surfactant may be preferred. The amount of such a surfactant is not specifically limited but is preferably from 0.01 to 20 wt.%.
   The gum solution has preferably a pH from 3 to 8, more preferably between 5 and 8, most preferably between 5 and 7. The pH of the gum solution is usually adjusted with a mineral acid, an organic acid or an inorganic salt in an amount of from 0.01 to 2 wt.%. Examples of the mineral acids include nitric acid, sulfuric acid, phosphoric acid and metaphosphoric acid. Especially organic acids are used as pH control agents and as desensitizing agents. Examples of the organic acids include carboxylic acids, sulfonic acids, phosphonic acids or salts thereof, e.g. succinates, phosphates, phosphonates, sulfates and sulfonates. Specific examples of the organic acid include citric acid, acetic acid, oxalic acid, malonic acid, p-toluenesulfonic acid, tartaric acid, malic acid, lactic acid, levulinic acid, phytic acid and organic phosphonic acid.
   The gum solution may also comprise an inorganic salt, preferably a mono or dibasic phosphate salt, more preferably an alkali-metal dihydrogen phosphate such as KH₂PO₄ or NaH₂PO₄.
   Examples of the inorganic salt include magnesium nitrate, monobasic sodium phosphate, dibasic sodium phosphate, nickel sulfate, sodium hexametaphosphate and sodium tripolyphosphate. Other inorganic salts can be used as corrosion inhibiting agents, e.g. magnesium sulfate or zinc nitrate. The mineral acid, organic acid or inorganic salt may be used singly or in combination with one or more thereof.
   The gum solution may also comprise a mixture of an anionic surfactant and an inorganic salt. In this mixture the anionic surfactant is preferably an anionic surfactant with a sulphonic acid group, more preferably an alkali-metal salt of a mono- or di-alkyl substituted diphenylether-sulphonic acid, and the inorganic salt is preferably a mono or dibasic phosphate salt, more preferably an alkali-metal dihydrogen phosphate, most preferably KH₂PO₄ or NaH₂PO₄.
   Besides the foregoing components, a wetting agent such as ethylene glycol, propylene glycol, triethylene glycol, butylene glycol, hexylene glycol, diethylene glycol, dipropylene glycol, glycerin, trimethylol propane and diglycerin may also be present in the gum solution. The wetting agent may be used singly or in combination with one or more thereof. In general, the foregoing wetting agent is preferably used in an amount of from 1 to 25 wt.%.
   Further, a chelate compound may be present in the gum solution. Calcium ion and other impurities contained in the diluting water can have adverse effects on printing and thus cause the contamination of printed matter. This problem can be eliminated by adding a chelate compound to the diluting water. Preferred examples of such a chelate compound include organic phosphonic acids or phosphonoalkanetricarboxylic acids. Specific examples are potassium or sodium salts of ethylenediaminetetraacetic acid, diethylenetriaminepentaacetic acid, triethylenetetraminehexaacetic acid, hydroxyethylethylenediaminetriacetic acid, nitrilotriacetic acid, 1-hydroxyethane-1,1-diphosphonic acid and aminotri(methylenephosphonic acid). Besides these sodium or potassium salts of these chelating agents, organic amine salts are useful. The preferred amount of such a chelating agent to be added is from 0.001 to 1.0 wt.% relative to the gum solution in diluted form.
   Further, an antiseptic and an anti-foaming agent may be present in the gum solution. Examples of such an antiseptic include phenol, derivatives thereof, formalin, imidazole derivatives, sodium dehydroacetate, 4-isothiazoline-3-one derivatives, benzoisothiazoline-3-one, benztriazole derivatives, amidineguanidine derivatives, quaternary ammonium salts, pyridine derivatives, quinoline derivatives, guanidine derivatives, diazine, triazole derivatives, oxazole and oxazine derivatives. The preferred amount of such an antiseptic to be added is such that it can exert a stable effect on bacteria, fungi, yeast or the like. Though depending on the kind of bacteria, fungi and yeast, it is preferably from 0.01 to 4 wt.% relative to the gum solution in diluted form. Further, preferably, two or more antiseptics may be used in combination to exert an aseptic effect on various fungi and bacteria. The anti-foaming agent is preferably silicone anti-foaming agents. Among these anti-foaming agents, either an emulsion dispersion type or solubilized type anti-foaming agent may be used. The proper amount of such an anti-foaming agent to be added is from 0.001 to 1.0 wt.% relative to the gum solution in diluted form.
   Besides the foregoing components, an ink receptivity agent may be present in the gum solution if desired. Examples of such an ink receptivity agent include turpentine oil, xylene, toluene, low heptane, solvent naphtha, kerosine, mineral spirit, hydrocarbons such as petroleum fraction having a boiling point of about 120°C to about 250°C, diester phthalates (e.g., dibutyl phthalate, diheptyl phthalate, di-n-octyl phthalate, di(2-ethylhexyl) phthalate, dinonyl phthalate, didecyl phthalate, dilauryl phthalate, butylbenzyl phthalate), aliphatic dibasic esters (e.g., dioctyl adipate, butylglycol adipate, dioctyl azelate, dibutyl sebacate, di(2-ethylhexyl) sebacate dioctyl sebacate), epoxidated triglycerides (e.g., epoxy soyabean oil), ester phosphates (e.g., tricresyl phosphate, trioctyl phosphate, trischloroethyl phosphate) and plasticizers having a solidification point of 15°C or less and a boiling point of 300°C or more at one atmospheric pressure such as esters of benzoates (e.g., benzyl benzoate). Examples of other solvents which can be used in combination with these solvents include ketones (e.g., cyclohexanone), halogenated hydrocarbons (e.g., ethylene dichloride), ethylene glycol ethers (e.g., ethylene glycol monomethyl ether, ethylene glycol monophenyl ether, ethylene glycol monobutyl ether), aliphatic acids (e.g., caproic acid, enathic acid, caprylic acid, pelargonic acid, capric acid, undecylic acid, lauric acid, tridecylic acid, myristic acid, pentadecylic acid, palmitic acid, heptadecylic acid, stearic acid, nonadecanic acid, arachic acid, behenic acid, lignoceric acid, cerotic acid, heptacosanoic acid, montanic acid, melissic acid, lacceric acid, isovaleric acid) and unsaturated aliphatic acids (e.g., acrylic acid, crotonic acid, isocrotonic acid, undecyclic acid, oleic acid, elaidic acid, cetoleic acid, erucic acid, butecidic acid, sorbic acid, linoleic acid, linolenic acid, arachidonic acid, propiolic acid, stearolic acid, clupanodonic acid, tariric acid, licanic acid). Preferably, it is an aliphatic acid which is liquid at a temperature of 50°C, more preferably has from 5 to 25 carbon atoms, most preferably has from 8 to 21 carbon atoms. The ink receptivity agent may be used singly or in combination with one or more thereof. The ink receptivity agent is preferably used in an amount of from 0.01 to 10 wt.%, more preferably from 0.05 to 5 wt.%. The foregoing ink receptivity agent may be present as an oil-in-water emulsion or may be solubilized with the aid of a solubilizing agent.
   The viscosity of the gum solution can be adjusted to a value of e.g. between 1.7 and 5 mPa.s (or cP), by adding viscosity increasing compounds, such as poly(ethylene oxide), e.g. having a molecular weight between 10⁵ and 10⁷. Such compounds can be present in a concentration of 0.01 to 10 g/l.
   A baking gum has a similar composition as described above, with the additional preference towards compounds that do not evaporate at the usual bake temperatures. Specific examples of suitable baking gum solutions are described in e.g. EP-A 222 297, EP-A 1 025 992, DE-A 2 626 473 and US 4,786,581.

### EXAMPLES

Preparation of the lithographic substrate.

A 0.30 mm thick aluminum foil was degreased by immersing the foil in an aqueous solution containing 40 g/l of sodium hydroxide at 60°C for 8 seconds and rinsed with demineralized water for 2 seconds. The foil was then electrochemically grained during 15 seconds using an alternating current in an aqueous solution containing 12 g/l of hydrochloric acid and 38 g/l of aluminum sulfate (18-hydrate) at a temperature of 33°C and a current density of 130 A/dm². After rinsing with demineralized water for 2 seconds, the aluminum foil was then desmutted by etching with an aqueous solution containing 155 g/l of sulfuric acid at 70°C for 4 seconds and rinsed with demineralized water at 25°C for 2 seconds. The foil was subsequently subjected to anodic oxidation during 13 seconds in an aqueous solution containing 155 g/l of sulfuric acid at a temperature of 45°C and a current density of 22 A/dm², then washed with demineralized water for 2 seconds and post-treated for 10 seconds with a solution containing 4 g/l of polyvinylphosphonic acid at 40°C, rinsed with demineralized water at 20°C during 2 seconds and dried.

The support thus obtained has a surface roughness Ra of 0.21 µm and an anodic weight of 4 g/m² of Al₂O₃.

Preparation of the printing plate precursors 1 - 2.

Printing plate precursors 1 and 2 were produced by applying a coating solution onto the above described lithographic substrate. The composition of the coating is defined in Table 1. The average particle sizes of the styrene/acrylonitrile copolymers were measured with a Brookhaven BI-90 analyzer, commercially available from Brookhaven Instrument Company, Holtsville, NY, USA, and are indicated in Table 2. The coating was applied from an aqueous coating solution and a dry coating weight of 0.8 g/m² was obtained.

**Table 1: composition of the dry coating (% wt)**

| INGREDIENTS | % wt |
|---|---|
| Polymer particle (1) | 77 |
| IR-2 (2) | 10 |
| Polyacrylic acid binder (3) | 10 |
| Cab O Jet 200 (4) | 3 |

(1) Polymer particle is copolymer of styrene/acrylonitrile, weight ratio 60/40, stabilized with an anionic wetting agent; average particle size as defined in Table 2;
(2) Infrared absorbing dye IR-2 has the following structure:
(3) Glascol D15 from ALLIED COLLOIDS, Mw = 2.7x10⁷ g/mol;
(4) Carbon dispersion in water from CABOT.

Imaging and processing of the printing plate precursors 1 - 2.

The plate precursors 1 and 2 were exposed with a Creo Trendsetter 2344T (40W) (plate-setter, trademark from CREO, Burnaby, Canada), operating at 150 rpm and varying energy densities up to 330 mJ/cm².

After imaging, the plate precursors were developed in a gumming unit, using Agfa RC520 (trademark from AGFA) as gumming solution. The RC520 solution is an aqueous solution of the surfactant DOWFAX 3B2, commercially available from DOW CHEMICAL, in a concentration of 39.3 g/l, citric acid.laq in a concentration of 9.8 g/l, and trisodium citrate.2aq in a concentration of 32.6 g/l, and the RC520 solution has a pH-value of about 5.

### Print results.

The plates were mounted on a GTO46 printing press (available from Heidelberger Druckmaschinen AG), and a print job was started using K + E Novavit 800 Skinnex ink (trademark of BASF Drucksysteme GmbH) and 3% FS101 (trademark of AGFA) in 10% isopropanol as fountain liquid.

The lithographic properties of the plates were determined by visual inspection of the clean-out in the non-exposed areas and the appearance of toning in the non-exposed areas on the press and by the run-length resistance (Table 2). A good run lenght resistance (+) means that after 100,000 prints the 2% highlight of a 200 lpi screen was still rendered on the print. An insufficient run lenght resistance (-) means that after 1,000 prints breakdown of the highlight of a 200 lpi screen occurred.

**Table 2: results of run-length and sensitivity.**

| Example number | Plate precursor | Average particle size nm | Sensitivity (*) (mJ/cm²) | Energy exposed (mJ/cm²) | Run length (**) |
|---|---|---|---|---|---|
| Invention Example 1 | Precursor 1 | 51 | 215 | 215 | + |
| | | | | 260 | + |
| | | | | 330 | + |
| Comparative Example 1 | Precursor 2 | 65 | 330 | 215 | - |
| | | | | 260 | - |
| | | | | 330 | + |

| | | | | | |
|---|---|---|---|---|---|
| (*) : energy required for a clear reproduction of a 2% dot of a 200 lpi screen on the printed copies; (**): see above. | | | | | |

The Invention Example 1 and the Comparative Example 1 show both an excellent clean-out and no toning. The results in Table 2 demonstrate that the Precursor 1, comprising a latex with an average particle size of 51 nm, has an improved sensitivity and a good run length. In the Comparative Example 1, the Precursor 2, comprising a latex with an average particle size of 65 nm, exhibits only a high run length with high exposure energy dose and has a reduced sensitivity.

### Preparation of the printing plate precursors 3 - 6.

Printing plate precursors 3 to 6 were produced by applying a coating solution onto the above described lithographic substrate. The composition of the coating is defined in Table 3. The average particle sizes of the styrene/acrylonitrile copolymers were measured with a Brookhaven BI-90 analyzer, commercially available from Brookhaven Instrument Company, Holtsville, NY, USA, and are indicated in Table 4. The coating was applied from an aqueous coating solution and a dry coating weight of 0.6 g/cm² was obtained.

**Table 3: composition of the dry coating (% wt)**

| INGREDIENTS | % wt |
|---|---|
| Polymer particle (1) | 77 |
| IR-2 (2) | 10 |
| Polyacrylic acid binder (3) | 10 |
| Cab O Jet 200 (4) | 3 |

| | |
|---|---|
| (1) Polymer particle is copolymer of styrene/acrylonitrile, weight ratio 60/40, stabilized with an anionic wetting agent; average particle size as defined in Table 4; (2) IR-2 as defined in Table 1; (3) Glascol D15 from ALLIED COLLOIDS; (4) Carbon dispersion in water from CABOT. | |

Imaging and processing of the printing plate precursors 3 - 6.

The plate precursors 3 - 6 were exposed with a Creo Trendsetter 2344T (40W) (plate-setter, trademark from CREO, Burnaby, Canada), operating at 150 rpm and varying energy densities up to 330 mJ/cm².

After imaging, the plate precursors were developed in a gumming unit, using Agfa RC520 (trademark from AGFA) as gumming solution.

### Print results.

The plates were mounted on a GT046 printing press (available from Heidelberger Druckmaschinen AG), and a print job was started using K + E Novavit 800 Skinnex ink (trademark of BASF Drucksysteme GmbH) and 3% FS101 (trademark of AGFA) in 10% isopropanol as fountain liquid.

The sensitivity, clean-out and toning were determined for these precursors as described in Invention Example 1 and are summarized in Table 4.

**Table 4: results of sensitivity and appearance of toning in the non-image areas of the plate.**

| Example number | Plate precursor | Average particle size nm | Sensitivity (*) (mJ/cm²) | Clean-out Behaviour (**) | Toning behaviour (***) |
|---|---|---|---|---|---|
| Comparative Example 2 | Precursor 3 | 36 | - | - | - |
| Invention Example 2 | Precursor 4 | 45 | 110 | + | + |
| Invention Example 3 | Precursor 5 | 50 | 150 | + | + |
| Invention Example 4 | Precursor 6 | 61 | 170 | + | + |

| | | | | | |
|---|---|---|---|---|---|
| (*) : energy required for a clear reproduction of a 2% dot of a 200 lpi screen on the printed copies; (**) : + indicates an excellent clean-out; - indicated an insufficient clean-out; (***) : + indicates no toning; - indicates toning. | | | | | |

The results in Table 4 demonstrate that the precursors, comprising a latex with an average particle size ≥ 45 nm, exhibit an excellent clean-out and no toning and a high sensitivity. In the Comparative Example 2, the Precursor 3, comprising a latex with a particle size of 36 nm, shows an insufficient clean-out and toning.

Preparation of the printing plate precursors 7 - 12.

The printing plate precursors 7 to 12 were produced by applying a coating onto the above described lithographic substrate. The composition of the coating is defined in Table 5. The coating was applied from an aqueous coating solution and a dry coating weight of 0.6 g/cm² was obtained.

**Table 5: Composition of the dry coating (%wt)**

| Plate precursor | Polymer particle (1) | IR-2 (2) | Binder (3) | Cab O Jet 250 (4) |
|---|---|---|---|---|
| Precursor 7 | 65% | 6% | 26% | 3% |
| Precursor 8 | 75% | 6% | 16% | 3% |
| Precursor 9 | 79% | 8% | 6% | 7% |
| Precursor 10 | 81% | 8% | 6% | 5% |
| Precursor 11 | 83% | 8% | 6% | 3% |
| Precursor 12 | 85% | 6% | 6% | 3% |

| | | | | |
|---|---|---|---|---|
| (1) Polymer particle is copolymer of styrene/acrylonitrile, weight ratio 60/40, stabilized with an anionic wetting agent; average particle size 51 nm, measured with a Brookhaven BI-90 analyzer, commercially available from Brookhaven Instrument Company, Holtsville, NY, USA; (2) IR-2 as defined in Table 1; (3) Glascol D15 from ALLIED COLLOIDS (4) Cu-Phtalocyanine-dispersion in water from CABOT. | | | | |

Imaging and processing of the printing plate precursors 7 - 12.

The plate precursors 7 - 12 were exposed with a Creo Trendsetter 2344T (40W) (plate-setter, trademark from CREO, Burnaby, Canada), operating at 150 rpm and varying energy densities up to 330 mJ/cm².

After imaging, the plate precursors were developed in a gumming unit, using Agfa RC520 (trademark from AGFA) as gumming solution.

### Print results.

The plates were mounted on a GTO46 printing press (available from Heidelberger Druckmaschinen AG) and a print job was started using K + E Novavit 800 Skinnex ink (trademark of BASF Drucksysteme GmbH) and 3% FS101 (trademark from Agfa) with 10% isopropanol as fountain liquid.

The sensitivity, clean-out and toning were determined for these precursors as described in Invention Example 1 and are summarized in Table 6.

**Table 6: results of sensitivity and appearance of toning in the non-image areas of the plate.**

| Example number | Plate precursor | Sensitivity (*) (mJ/cm²) | Clean-out behaviour (**) | Toning behaviour (***) |
|---|---|---|---|---|
| Comparative Example 3 | Precursor 7 | 330 | + | + |
| Invention Example 5 | Precursor 8 | 190 | + | + |
| Invention Example 6 | Precursor 9 | 190 | + | + |
| Invention Example 7 | Precursor 10 | 190 | + | + |
| Invention Example 8 | Precursor 11 | 190 | + | + |
| Comparative Example 4 | Precursor 12 | - | - | - |

| | | | | |
|---|---|---|---|---|
| (*) : energy required for a clear reproduction of a 2% dot of a 200 lpi screen on the printed copies; (**) : + indicates an excellent clean-out; - indicated an insufficient clean-out; (***): + indicates no toning; - indicates toning. | | | | |

The results in Table 6 demonstrate that the precursors, comprising a latex of 51 nm in an amount of < 85 % wt, exhibit an excellent clean-out and no toning, but a high sensitivity is only obtained for an amount of the latex > 65 % wt, namely for the Precursor 7, comprising 65 % wt of the latex, a sensitivity of 330 mJ/m² is obtained.

Preparation of the printing plate precursors 13 - 16.

The printing plate precursors 13 to 16 were produced in the same way as the precursors 7 to 12 with the exception that the Cab O Jet 250 is replaced by Cap O Jet 200 in the same amounts. The composition of the coating for the precursors 13 to 16 is defined in Table 7. The coating was applied from an aqueous coating solution onto the above described lithographic substrate, and a dry coating weight of 0.6 g/cm² was obtained.

**Table 7: composition of the dry coating (%wt)**

| Plate precursor | Polymer particle (1) | IR-2 (2) | Binder (3) | Cab O Jet 200 (4) |
|---|---|---|---|---|
| Precursor 13 | 65% | 6% | 26% | 3% |
| Precursor 14 | 75% | 6% | 16% | 3% |
| Precursor 15 | 83% | 8% | 6% | 3% |
| Precursor 16 | 85% | 6% | 6% | 3% |

| | | | | |
|---|---|---|---|---|
| (1) Polymer particle is copolymer ot styrene/acrylonitrile, weight ratio 60/40, stabilized with an anionic wetting agent; average particle size of 51 nm, measured with a Brookhaven BI-90 analyzer, commercially available from Brookhaven Instrument Company, Holtsville, NY, USA; (2) IR-2 as defined in Table 1; (3) Glascol D15 from ALLIED COLLOIDS; (4) Carbon dispersion in water from CABOT. | | | | |

Imaging and processing of the printing plate precursors 13 - 16.

The plate precursors 13 - 16 were exposed and processed in an identical way as defined above for the precursors 7 - 12.

### Print results.

The plates were mounted on a GT046 printing press (available from Heidelberger Druckmaschinen AG) and a print job was started using K + E Novavit 800 Skinnex ink (trademark of BASF Drucksysteme GmbH) and 3% FS101 (trademark from AGFA) with 10% isopropanol as fountain liquid.

The sensitivity, clean-out and toning were determined for these precursors as described in Invention Example 1 and are summarized in Table 8.

**Table 8: results of sensitivity and appearance of toning in the non-image areas of the plate.**

| Example number | Plate precursor | Sensitivity (*) (mJ/cm²) | Clean-out behaviour (**) | Toning behaviour (***) |
|---|---|---|---|---|
| Comparative Example 5 | Precursor 13 | 330 | + | + |
| Invention Example 9 | Precursor 14 | 210 | + | + |
| Invention Example 10 | Precursor 15 | 190 | + | + |
| Comparative Example 6 | Precursor 16 | - | - | + |

| | | | | |
|---|---|---|---|---|
| (*) : energy required for a clear reproduction of a 2% dot of a 200 lpi screen on the printed copies; (**) : + indicates an excellent clean-out; - indicated an insufficient clean-out; (***): + indicates no toning; - indicates toning. | | | | |

The results in Table 8 demonstrate that the precursors, comprising a latex of 51 nm in an amount of < 85 % wt, exhibit an excellent clean-out and no toning, but a high sensitivity is only obtained for an amount of the latex > 65 % wt, namely for the Precursor 13, comprising 65 % wt of the latex, a sensitivity of 330 mJ/m² is obtained.

## Claims

1. A method of making a lithographic printing plate comprising the steps of:
- providing a lithographic printing plate precursor comprising
(i) a support having a hydrophilic surface or which is provided with a hydrophilic layer;
(ii) on said support, a coating comprising an image recording layer, said layer comprising hydrophobic thermoplastic polymer particles and a hydrophilic binder, said coating further comprising a pigment, present in said image recording layer or in an additional layer of said coating;
- image-wise exposing said coating, thereby inducing coalescence of the thermoplastic polymer particles at the exposed areas of the image recording layer;
- developing the precursor by applying a gum solution to the coating, thereby removing the non-exposed areas of the image recording layer from the support, and
- optionally, baking the developed precursor;
**characterized in that** said hydrophobic thermoplastic polymer particles have an average particle size between 40 nm and 63 nm, and that the amount of the hydrophobic thermoplastic polymer particles is more than 70 % and less than 85 % by weight, relative to the image recording layer, and
that said pigment has a hydrophilic surface and provides a visible image after image-wise exposing and developing with the gum solution.

2. A method according to claim 1 wherein said particles have an average particle size between 45 nm and 63 nm.

3. A method according to claim 1 wherein said particles have an average particle size between 45 nm and 59 nm.

4. A method according to any of preceding claims wherein the amount of the hydrophobic thermoplastic polymer particles ranges from 75 to 84 % by weight, relative to the image recording layer.

5. A method according to any of preceding claims wherein the amount of the hydrophobic thermoplastic polymer particles ranges from 77 to 83 % by weight, relative to the image recording layer.

6. A method according to any of preceding claims wherein the coating weight of said image recording layer ranges between 0.45 and 0.85 g/m².

7. A method according to any of preceding claims wherein the coating weight of said image recording layer ranges between 0.50 and 0.80 g/m2..

8. A method according to any of preceding claims wherein the coating weight of said image recording layer ranges between 0.55 and 0.75 g/m².

9. A method according to any of preceding claims wherein said hydrophobic thermoplastic polymer particles comprise a copolymer of styrene and acrylonitrile or methacrylonitrile.

10. A method according to any of preceding claims wherein said coating further comprises an IR-absorbing agent.

11. A method according to claim 10 wherein said IR-absorbing agent is present in said image-recording layer in an amount of at least 6 % by weight relative to the image-recording layer.

12. A method according to any of preceding claims wherein said pigment has hydrophilic groups on the surface.

13. A method according to claim 12 wherein said hydrophilic groups are anionic or non-ionic groups.

14. A method according to any of preceding claims wherein said gum solution contains a hydrophilic film-forming polymer and/or surfactant and wherein the pH of said gum solution ranges between 3 and 8.

15. A method according to any of preceding claims wherein said developing is carried out in a gumming unit which is provided with at least one roller for rubbing and/or brushing the coating during development.

16. A method according to claim 15 wherein the image-wise exposing step is carried out in a plate setter which is mechanically coupled to the gumming unit by conveying means.

17. A method according to claim 15 or 16 wherein said optionally baking step is carried out in a baking unit which is mechanically coupled to the gumming unit by conveying means.

## Patentansprüche

1. Ein Verfahren zur Herstellung einer lithografischen Druckplatte, das folgende Schritte umfasst :
Bereitstellen einer lithografischen Druckplattenvorstufe, umfassend :
(i) einen Träger mit einer hydrophilen Oberfläche oder einen mit einer hydrophilen Schicht versehenen Träger,
(ii) eine auf den Träger angebrachte Beschichtung, die eine Teilchen eines hydrophoben thermoplastischen Polymers und ein hydrophiles Bindemittel enthaltende Bildaufzeichnungsschicht umfasst, wobei die Beschichtung ferner ein in der Bildaufzeichnungsschicht oder in einer zusätzlichen Schicht der Beschichtung enthaltenes Pigment enthält,
- bildmäßige Belichtung der Beschichtung, wodurch ein Koaleszieren der Teilchen eines thermoplastischen Polymers in den belichteten Bereichen der Bildaufzeichnungsschicht ausgelöst wird,
- Entwicklung der Vorstufe durch Auftrag einer Gummierlösung auf die Beschichtung, wobei die nicht-belichteten Bereiche der Bildaufzeichnungsschicht vom Träger entfernt werden, und
- eventuelles Einbrennen der entwickelten Vorstufe,
**dadurch gekennzeichnet, dass** die Teilchen eines hydrophoben thermoplastischen Polymers eine mittlere Teilchengröße zwischen 40 nm und 63 nm aufweisen,
und die Menge der Teilchen eines hydrophoben thermoplastischen Polymers mehr als 70 Gew.-% und weniger als 85 Gew.-%, bezogen auf die Bildaufzeichnungsschicht, beträgt, und
das Pigment eine hydrophile Oberfläche hat und nach bildmäßiger Belichtung und Entwicklung mit der Gummierlösung ein sichtbares Bild ergibt.

2. Verfahren nach Anspruch 1, **dadurch gekennzeichnet, dass** die Teilchen eine mittlere Teilchengröße zwischen 45 nm und 63 nm aufweisen.

3. Verfahren nach Anspruch 1, **dadurch gekennzeichnet, dass** die Teilchen eine mittlere Teilchengröße zwischen 45 nm und 59 nm aufweisen.

4. Verfahren nach einem der vorstehenden Ansprüche, **dadurch gekennzeichnet, dass** die Menge der Teilchen eines hydrophoben thermoplastischen Polymers zwischen 75 Gew.-% und 84 Gew.-%, bezogen auf die Bildaufzeichnungsschicht, liegt.

5. Verfahren nach einem der vorstehenden Ansprüche, **dadurch gekennzeichnet, dass** die Menge der Teilchen eines hydrophoben thermoplastischen Polymers zwischen 77 Gew.-% und 83 Gew.-%, bezogen auf die Bildaufzeichnungsschicht, liegt.

6. Verfahren nach einem der vorstehenden Ansprüche, **dadurch gekennzeichnet, dass** das Auftragsgewicht der Bildaufzeichnungsschicht zwischen 0,45 g/m² und 0,85 g/m² liegt.

7. Verfahren nach einem der vorstehenden Ansprüche, **dadurch gekennzeichnet, dass** das Auftragsgewicht der Bildaufzeichnungsschicht zwischen 0,50 g/m² und 0,80 g/m² liegt.

8. Verfahren nach einem der vorstehenden Ansprüche, **dadurch gekennzeichnet, dass** das Auftragsgewicht der Bildaufzeichnungsschicht zwischen 0,55 g/m² und 0,75 g/m² liegt.

9. Verfahren nach einem der vorstehenden Ansprüche, **dadurch gekennzeichnet, dass** die Teilchen eines hydrophoben thermoplastischen Polymers ein Copolymer aus Styrol und Acrylnitril oder Methacrylnitril enthalten.

10. Verfahren nach einem der vorstehenden Ansprüche, **dadurch gekennzeichnet, dass** die Beschichtung ferner einen IR-Absorber enthält.

11. Verfahren nach Anspruch 10, **dadurch gekennzeichnet, dass** die Menge des IR-Absorbers in der Bildaufzeichnungsschicht mindestens 6 Gew.-%, bezogen auf die Bildaufzeichnungsschicht, beträgt.

12. Verfahren nach einem der vorstehenden Ansprüche, **dadurch gekennzeichnet, dass** die Oberfläche des Pigments hydrophile Gruppen enthält.

13. Verfahren nach Anspruch 12, **dadurch gekennzeichnet, dass** die hydrophilen Gruppen anionische Gruppen oder nicht-ionische Gruppen sind.

14. Verfahren nach einem der vorstehenden Ansprüche, **dadurch gekennzeichnet, dass** die Gummierlösung ein hydrophiles filmbildendes Polymer und/oder ein Tensid enthält und der pH der Gummierlösung zwischen 3 und 8 variiert.

15. Verfahren nach einem der vorstehenden Ansprüche, **dadurch gekennzeichnet, dass** die Entwicklung in einer Gummiereinheit, die mit zumindest einer die Beschichtung während der Entwicklung wischenden und/oder bürstenden Walze ausgestattet ist, stattfindet.

16. Verfahren nach Anspruch 15, **dadurch gekennzeichnet, dass** der Schritt der bildmäßigen Belichtung in einem mechanisch mittels Fördermitteln an die Gummiereinheit angekuppelten Plattenbelichter stattfindet.

17. Verfahren nach Anspruch 15 oder 16, **dadurch gekennzeichnet, dass** der eventuelle Einbrennschritt in einer mechanisch mittels Fördermitteln an die Gummiereinheit angekuppelten Einbrenneinheit stattfindet.

## Revendications

1. Un procédé pour la confection d'une plaque d'impression lithographique, comprenant les étapes ci-après :
- la mise à disposition d'un précurseur de plaque d'impression lithographique, comprenant :
(i) un support ayant une surface hydrophile ou un support revêtu d'une couche hydrophile,
(ii) un revêtement appliqué sur le support, comprenant une couche d'enregistrement d'image contenant des particules d'un polymère thermoplastique hydrophobe et un liant hydrophile, ledit revêtement contenant en outre un pigment contenu dans la couche d'enregistrement d'image ou dans une couche supplémentaire du revêtement,
- l'exposition sous forme d'image du revêtement, provoquant la coalescence des particules d'un polymère thermoplastique dans les zones exposées de la couche d'enregistrement d'image,
- le développement du précurseur en appliquant une solution de gommage sur le revêtement, permettant d'éliminer du support les zones non exposées de la couche d'enregistrement d'image, et
- la cuisson éventuelle du précurseur développé,
**caractérisé en ce que** les particules d'un polymère thermoplastique hydrophobe présentent une grandeur de particule moyenne comprise entre 40 nm et 63 nm,
et que la quantité des particules d'un polymère thermoplastique hydrophobe est supérieure à 70% en poids et inférieure à 85% en poids par rapport à la couche d'enregistrement d'image, et
que le pigment a une surface hydrophile et génère une image visible après l'exposition sous forme d'image et le développement en utilisant la solution de gommage.

2. Procédé selon la revendication 1, **caractérisé en ce que** les particules présentent une grandeur de particule moyenne comprise entre 45 nm et 63 nm.

3. Procédé selon la revendication 1, **caractérisé en ce que** les particules présentent une grandeur de particule moyenne comprise entre 45 nm et 59 nm.

4. Procédé selon l'une quelconque des revendications précédentes,
**caractérisé en ce que** la quantité des particules d'un polymère thermoplastique hydrophobe est comprise entre 75% en poids et 84% en poids par rapport à la couche d'enregistrement d'image.

5. Procédé selon l'une quelconque des revendications précédentes,
**caractérisé en ce que** la quantité des particules d'un polymère thermoplastique hydrophobe est comprise entre 77% en poids et 83% en poids par rapport à la couche d'enregistrement d'image.

6. Procédé selon l'une quelconque des revendications précédentes,
**caractérisé en ce que** le grammage de la couche d'enregistrement d'image est compris entre 0,45 g/m² et 0,85 g/m².

7. Procédé selon l'une quelconque des revendications précédentes,
**caractérisé en ce que** le grammage de la couche d'enregistrement d'image est compris entre 0,50 g/m² et 0,80 g/m².

8. Procédé selon l'une quelconque des revendications précédentes,
**caractérisé en ce que** le grammage de la couche d'enregistrement d'image est compris entre 0,55 g/m² et 0,75 g/m².

9. Procédé selon l'une quelconque des revendications précédentes,
**caractérisé en ce que** les particules d'un polymère thermoplastique hydrophobe comprennent un copolymère de styrène et d'acrylonitrile ou de méthacrylonitrile.

10. Procédé selon l'une quelconque des revendications précédentes,
**caractérisé en ce que** le revêtement contient en outre un agent absorbant les rayons infrarouges.

11. Procédé selon la revendication 10, **caractérisé en ce que** la quantité minimale de l'agent absorbant les rayons infrarouges dans la couche d'enregistrement d'image s'élève à 6% en poids par rapport à la couche d'enregistrement d'image.

12. Procédé selon l'une quelconque des revendications précédentes, **caractérisé en ce que** la surface du pigment contient des groupes hydrophiles.

13. Procédé selon la revendication 12, **caractérisé en ce que** les groupes hydrophiles sont des groupes anioniques ou des groupes non ioniques.

14. Procédé selon l'une quelconque des revendications précédentes, **caractérisé en ce que** la solution de gommage contient un polymère hydrophile filmogène et/ou un agent tensioactif et que le pH de la solution de gommage varie entre 3 et 8.

15. Procédé selon l'une quelconque des revendications précédentes, **caractérisé en ce que** le développement est effectué dans une unité de gommage munie d'au moins un rouleau servant à frotter et/ou à brosser le revêtement pendant le processus de développement.

16. Procédé selon la revendication 15, **caractérisé en ce que** l'étape de l'exposition sous forme d'image est effectuée dans une unité d'exposition directe de plaques mécaniquement accouplée à l'unité de gommage par des moyens de transport.

17. Procédé selon la revendication 15 ou 16, **caractérisé en ce que** l'étape éventuelle de la cuisson est effectuée dans une unité de cuisson mécaniquement accouplée à l'unité de gommage par des moyens de transport.
